

Feb. 4, 1936.

G. L. PARKHURST

2,029,689

SOLVENT FRACTIONATION

Filed April 29, 1933



## UNITED STATES PATENT OFFICE

2,029,689

## SOLVENT FRACTIONATION

George L. Parkhurst, Chicago, Ill., assignor to  
 Standard Oil Company, Chicago, Ill., a corpora-  
 tion of Indiana

Application April 29, 1933, Serial No. 668,593

8 Claims. (Cl. 196—37)

This invention relates to the solvent fractionation of petroleum materials and particularly lubricating oils and lubricating oil stocks. It further relates to the combined solvent fractionation of lubricating oils and naphthas.

It is an object of the invention to produce higher yields of improved lubricating oils than is possible by existing methods and/or to produce better products than do existing methods. The objects of the invention will become apparent in detail as the description thereof proceeds.

It has long been known to fractionate lubricating oil stocks by means of liquid sulfur dioxide. In these processes the more desirable paraffinic and naphthenic compounds are left undissolved and form the "raffinate", whereas the less desirable aromatic and olefinic constituents are dissolved by the sulfur dioxide and form the "extract". The raffinate fraction is, in general, characterized by a lower temperature co-efficient of viscosity, lower carbon forming tendency and greater sludge and oxidation stabilities than the original lubricating oil stock.

I have now found that these improved characteristics of the raffinate are very materially enhanced by the addition to the liquid sulfur dioxide of low boiling olefinic hydrocarbons such as are contained in cracked petroleum naphthas and particularly in those petroleum naphthas produced by vapor phase cracking processes. By variations in operating conditions particularly temperature, composition of the mixed solvent and ratio of solvent to material being extracted, it is possible to utilize the advantages of my process either by producing a better raffinate than can be done by means of liquid sulfur dioxide alone or alternatively produce a higher yield of raffinate similar to that produced by prior art processes. The optimum operating conditions can be readily determined by experiment in each particular case.

My invention can best be described by reference to the accompanying drawing which represents a conventional flow diagram of a process for the utilization of my invention. A petroleum material, preferably a lubricating oil stock, is introduced into mixer 11 by means of line 12. Simultaneously, a cracked naphtha, preferably produced by a vapor phase cracking process, is introduced into mixer 11 through line 13. Liquid sulfur dioxide can also be introduced directly at this point but I prefer to introduce an extract fraction from a subsequent stage in the process. This fraction contains a high percentage of liquid sulfur dioxide and is introduced into mixer 11 by

means of line 14. These various materials can be cooled, either prior to or subsequent to mixing, to the temperature desired for the fractionation operation. Cooling means are not specifically shown,—cooling may be effected by exchangers or it may be obtained by the vaporization of a portion of the sulfur dioxide. The mixed materials from mixer 11 pass through line 15 into separator 16 wherein extract and raffinate fractions separate, the former being withdrawn through line 17 and the latter through line 18. The extract fraction will be found to contain the undesirable constituents of the lubricating oil stock, namely the naphthenic and aromatic constituents together with a naphtha fraction which has a high antiknock value (high octane number) due to its high percentage of olefinic constituents as compared with the portion of the original naphtha passing out of settler 16 through line 18.

The extract is withdrawn through line 17 by means of pump 18 into bubble tower 19 wherein the lubricating oil constituents, naphtha constituents and sulfur dioxide are separated by fractional distillation. The oil extract containing undesirable lubricating oil constituents is removed from the bottom of tower 19 through line 20 and valve 21. A steam coil 22 in the base of tower 19 provides reboiling and prevents the withdrawal of naphtha constituents at this point. At an intermediate level in the tower above the point at which the extract is introduced, a special trap-out plate 23 is provided and the condensate at that point is withdrawn through line 24 and introduced into stripping column 25, the gasoline constituents being withdrawn from the base of the stripping column by means of line 26. A small amount of reboiling may be provided by means of closed steam coil 27. Any sulfur dioxide in the material removed through line 24 is returned to the main tower 19 by means of line 28. Cooling at the top of tower 19 is provided by means of dephlegmating coil 29. Sulfur dioxide passes off in vapor form from the top of the tower through line 30, passes through compressor 31 and is cooled and/or condensed by means of cooling coil 32, passing into storage tank 33 in liquid form.

Returning to the raffinate fraction removed from settler 16 by means of line 18 it is pumped (if necessary) by means of pump 34 into mixer 35, at which point it is mixed with the extract fraction from the third stage of the process introduced through line 36. The mixed material passes through line 37 into a second settler 38, wherein extract and raffinate fractions are again

formed. The former, is removed from separator 38 through valve 39, pump 40 and line 14 into mixer 41. A portion of the high octane number naphtha fraction from stripping tower 25 can also be introduced at this point by means of line 41 and valve 42, the remainder being withdrawn from the process through valve 43. By recycling at least a part of this high octane number naphtha fraction in which the olefinic hydrocarbons present in the original naphtha stock have been concentrated it is possible to increase the olefine content of the naphtha present in the various stages of the process and thereby increase the efficiency of the solvent fractionation of the lubricating oil. By means of valves 42a and 42b it is also possible to increase in a direct manner the olefinic hydrocarbon content of the mixed solvent present in the second and third stages, respectively.

20 The raffinate from separator 38 which contains a higher grade of lubricating oil constituents than did the raffinate from separator 16 is pumped (if necessary) by means of pump 44 into mixer 45, wherein it is mixed with fresh liquid 25 sulfur dioxide introduced from storage tank 33 by means of pump 46. The mixed materials pass through line 47 into a third separator 48 wherein extract and raffinate fractions are again formed. The former, containing an intermediate 30 grade of lubricating oil constituents, is recycled by means of pump 49 to an intermediate point in the process, preferably to mixer 35 preceding the second stage of the extraction. The raffinate fraction from separator 48 contains lubricating 35 oil constituents which have been extracted three times and which contain little or nothing except the highly desirable paraffinic and in some instances, naphthenic constituents. This raffinate is removed through line 50 by means of pump 51 40 and is introduced into bubble tower 52 which is generally similar to bubble tower 19 and contains trap-out plate 53, dephlegmating coil 54 and re-boiling coil 55 corresponding respectively to elements 23, 29 and 21 in tower 19. The raffinate 45 from which gasoline constituents and sulfur dioxide have been removed is drawn off at the base of tower 52 through valve 56 and passes to subsequent refining operations or to storage. Condensate is withdrawn from trap-out plate 53 into stripping column 57 corresponding to stripping column 25. The gasoline constituents are removed from the base of column 57 through valve 58. The naphtha fraction removed at this point is a relatively paraffinic fraction and is characterized by a low octane number. It may be used as a low grade gasoline or as a special naphtha or it may be subjected to a pyrolytic "reforming" 55 process to raise its octane number. Sulfur dioxide is removed from stripping column 57 through line 58 and is re-introduced into tower 52. Sulfur dioxide passes from the top of tower 52 in vapor form through line 59, compressor 60 and cooling and/or condensing coil 61 into storage tank 33 from which it is subsequently re-introduced into the process.

It will be seen from the foregoing description that by means of a three-stage process the advantages of counter-current extraction have been obtained. Thus the material passing into separator 16 contains, in addition to fresh lubricating oil stock, fresh naphtha and a lubricating oil extract which has twice had its raffinate fractions removed. The saturated constituents of the naphtha, having a relatively high solvent power for oil, remove practically all of the more valuable

5 lubricating oil constituents and prevent them from passing out of the process through line 17. In the second stage of the process, that is, in separator 38, the ratio of sulfur dioxide to naphtha has been raised by the removal of a highly olefinic portion of the naphtha through line 17 and by the introduction of the extract from the third stage of the process which is high in sulfur dioxide. The result is that an increased amount of the paraffinic and naphthenic lubricating oil constituents appear in the raffinate from this second 10 stage of the process. In the third stage, that is, in separator 48 the sulfur dioxide-naphtha ratio is again increased, this time by the introduction of fresh liquid sulfur dioxide, and a maximum 15 amount of the olefinic constituents of the naphtha is removed and recycled to the second stage.

A special feature of my process resides in the fact that at one and the same time I am able to fractionate a lubricating oil stock into a relatively high grade and a relatively low grade fraction and fractionate an olefinic naphtha into a high octane number fraction and a low octane number fraction. In typical instances I can produce from 40 to 90% of an extract lubricating 20 oil fraction having a viscosity-gravity constant (Industrial and Engineering Chemistry, volume 24, page 1371, December, 1932) from .01 to .07 lower than that of the original lubricating oil stock and from .01 to .03 lower than that of the 25 raffinate fraction produced by the use of liquid sulfur dioxide alone. Simultaneously I produce from 15 to 60% of an extract naphtha fraction having an octane number (National Petroleum News, June 4, 1930; page 35) from 3 to 20 points 30 higher than that of the original naphtha stock.

It will be readily comprehended that this process can be used on a variety of petroleum materials such as gas oil and lubricating oils, under a variety of operating conditions. As a preferred embodiment, I treat the total lubricating oil fraction from the distillation of Mid-Continent petroleum with an olefinic cracked naphtha produced by vapor phase cracking and lying preponderantly within the gasoline boiling point range. The temperature 40 of the extraction is preferably between 0° and 50° F., although much lower temperatures and somewhat higher temperatures can be used if desired. Throughout most of the preferred temperature range the system should be held under pressure, 45 but if it is desired to operate at low temperatures this can be done by partially exhausting at each stage of the process. The temperature of each stage can be varied by varying the pressure from point to point and/or by the use of heaters and/or coolers. It is also sometimes desirable to heat the various materials prior to or during the mixing steps and then to cool them to enhance separation 50 into extract and raffinate fractions.

The olefinic naphtha used in my process may be 55 a pressure distillate, particularly a pressure distillate from a vapor phase cracking process. Olefinic gasolines, refined or unrefined, can also be used. It is generally advantageous, however, to use a cracked heavy naphtha, for instance, a 60 naphtha boiling between 250° F. and 450° F. The use of a naphtha of this type increases the ease of separation of sulfur dioxide from the naphtha, lowers naphtha losses and increases the efficiency 65 of the naphtha fractionation since the low boiling constituents are in general already high in octane number. As one example of such a cracked heavy naphtha, I may use a vapor phase cracked naphtha boiling between 250° F. and 450° F. and con- 70

taining approximately 52% olefines, 1% aromatics and 47% paraffins and naphthenes.

In one modification of my invention I extract the naphtha initially with liquid sulfur dioxide and employ only the extract portion in my lubricating oil refining process. I may use a cracked heavy naphtha or other low boiling hydrocarbon mixture containing olefinic hydrocarbons, such as cracked gasoline or liquefied hydrocarbons recovered from cracking still gases. On treating such a naphtha with liquid sulfur dioxide at temperatures below the miscibility temperature, an extract is obtained which may be used directly in my lubricating oil fractionation process without elimination of the sulfur dioxide contained in the naphtha extract. After the unsaturated hydrocarbon material has performed its function in the extraction of undesirable constituents from the lubricating oil, it may be recovered and re-used, or it may be discharged from the process and used as a high octane number motor fuel or blended with other materials in the manufacture of such a motor fuel.

Although I prefer to use a counter-current process as described, it will be understood that a batch process in which the liquid sulfur dioxide, olefinic material and lubricating oil stock are co-agitated below the miscibility temperature or a batch process in which these materials are put into solution and then separated into raffinate and extract fraction by cooling can be used.

The principal requisite of the olefinic material used in my process is the presence of substantial amounts, preferably at least 25%, of an olefinic hydrocarbon or olefinic hydrocarbons boiling below about 400° F. and preferably below 350° F. Higher boiling olefines are unsuitable.

Instead of using cracked naphtha I can obtain the same beneficial results insofar as the improvement of the lubricating oil stock is concerned by the use of pure olefinic hydrocarbons or mixtures of these. As examples, I may use ethylene, propylene, butylene, or amylene or their mixtures as they occur naturally in cracking still gases. Using these low boiling olefines has the advantage of permitting low operating temperatures without the use of sub-atmospheric pressures.

The ratio of olefinic hydrocarbon or naphtha to liquid sulfur dioxide will obviously vary with the type of material it is intended to extract and the desired degree of extraction. In general, I prefer to use about one volume of olefinic material to from 2 to 5 volumes of liquid sulfur dioxide but ratios as low as one volume of olefinic material to 20 of sulfur dioxide show some advantage over liquid sulfur dioxide alone and ratios as high as one-to-one or even higher can be used under some conditions.

The ratio of the total volume of liquid sulfur dioxide and olefinic material to the volume of lubricating oil stock or other petroleum material to be extracted can be varied within wide limits but preferably between 1 volume of mixed solvent to 2 volumes of oil and 5 volumes of mixed solvent to 1 volume of oil.

Insofar as the simultaneous solvent fractionation of a lubricating oil stock and an olefinic naphtha stock is concerned it will be understood that my invention is not restricted to the use of liquid sulfur dioxide but that other selective sol-

vents such as methyl alcohol, acetone, aniline or liquid carbon dioxide can be used in place of liquid sulfur dioxide. These alternative solvents are, however, in one way or another generally inferior to sulfur dioxide.

Although I have described my invention in terms of certain specific embodiments thereof, it will be readily comprehended that numerous modifications fall within its scope and I do not wish to be limited except to the subject matter of the appended claims.

I claim:

1. In the solvent fractionation of a lubricating oil stock the steps which comprise mixing said stock with a substantial amount of liquid sulfur dioxide and a substantial amount of a vapor phase cracked naphtha containing at least 25% olefins and separately recovering an extract fraction and a raffinate fraction. 15

2. Steps according to claim 1 in which said naphtha is a heavy naphtha boiling between 20 about 250° F. and about 450° F.

3. In the solvent fractionation of a lubricating oil stock the steps which comprise mixing said stock with a substantial amount of liquid sulfur dioxide and a substantial amount of a vapor phase cracked naphtha containing approximately 52% olefines and separately recovering an extract fraction and a raffinate fraction. 25

4. Steps according to claim 3 in which said naphtha is a heavy naphtha boiling between 30 about 250° F. and about 450° F.

5. In the solvent fractionation of a lubricating oil stock the steps which comprise mixing said stock with a substantial amount of liquid sulfur dioxide and a substantial amount of a solvent extract from a vapor phase cracked naphtha, said solvent extract containing at least about 25% olefins and separately recovering an extract fraction and a raffinate fraction. 35

6. In the solvent fractionation of a lubricating oil stock the steps which comprise mixing said stock with a substantial amount of liquid sulfur dioxide and a substantial amount of a vapor phase cracked naphtha containing at least 25% olefins 45 boiling below about 400° F. and separately recovering an extract fraction and a raffinate fraction.

7. In the solvent fractionation of a lubricating oil stock the steps which comprise mixing said stock with a substantial amount of liquid sulfur dioxide and a substantial amount of a vapor phase cracked naphtha containing at least 25% olefins boiling below about 350° F. and separately recovering an extract fraction and a raffinate fraction. 55

8. In the solvent fractionation of a lubricating oil stock the steps which comprise mixing said stock with a mixed solvent comprising liquid sulfur dioxide and a vapor phase cracked naphtha containing at least about 25% olefins, in a proportion between one volume of mixed solvent to two volumes of said stock and five volumes of mixed solvent to one volume of said stock, said mixed solvent comprising said sulfur dioxide and said vapor phase cracked naphtha in a proportion of one volume of said vapor phase cracked naphtha to from two to five volumes of said liquid sulfur dioxide, and separately recovering an extract fraction and a raffinate fraction. 65